

## UNITED STATES PATENT OFFICE

2,252,666

WAX-SUBSTITUTED ARYL ETHER ACIDS  
AND METHOD OF MAKING SAME

Orland M. Reiff, Woodbury, N. J., and Ferdinand P. Otto, Philadelphia, Pa., assignors to Socony-Vacuum Oil Company, Incorporated, New York, N. Y., a corporation of New York

No Drawing. Application August 26, 1938,  
Serial No. 226,910

13 Claims. (Cl. 260—521)

This invention relates to the production of certain new chemical compounds or compositions which may be generally designated as wax-substituted aryl ether acids. Although the invention is broadly concerned with chemical compounds or compositions coming within the above designated general classification, it contemplates as a preferred group within such general classification those compounds or compositions which are soluble or miscible with mineral oil.

Our invention is based upon the discovery that the oil-miscible wax-substituted aryl ether acids are of multifunctional activity when blended with viscous mineral oil fractions in that they effect improvement of several unrelated and related properties of the oil. For example, this preferred oil-miscible group of compounds or compositions coming within the general field of invention contemplated herein are effective, when blended in a minor proportion with viscous mineral oil fractions, such as mineral oil fractions of the lubricant type, to depress the pour point and improve the viscosity index of the oil. The present invention, however, is not concerned with the mineral oil composition obtained by blending a compound of the type contemplated herein with oil. Such mineral oil compositions form the subject matter of our copending application Serial No. 226,911, filed August 26, 1938 (now Patent 2,198,293), to which reference is made for further details in the composition of these preferred oil-miscible compounds.

It is to be understood, therefore, that while our invention contemplates oil-miscible compounds or compositions of the type referred to above, as a preferred class or group within the general field of invention, the invention is not limited to such oil-miscible compounds or compositions, since the whole class of new materials is possessed of valuable properties irrespective of oil miscibility. For example, these compounds or compositions may be used as intermediaries in the production of the corresponding metal salts, resins, resin-like materials, rubber substitutes, etc. Numerous other uses and applications of the compound or compositions contemplated herein will be readily apparent to those skilled in the art from the following description of their composition and preferred methods of synthesis.

The compounds or compositions contemplated by this invention may be broadly classified as wax or heavy alkyl substituted aryl ether acids. They may also be characterized as hydroxyaromatic (phenolic) compounds in which part of the nuclear hydrogen has been replaced with an aliphatic hydrocarbon group or groups derived from a high molecular weight aliphatic or pre-

dominantly aliphatic material, and in which the hydroxyl hydrogen has been replaced with an organic aliphatic or aromatic carboxylic acid group, (the aliphatic type comprising fatty and alicyclic acids; the aromatic comprising benzoid and heterocyclic acids).

The term "heavy alkyl" or "wax" as used herein in connection with the alkyl substituents on the characterizing aryl nuclei of these ether acids 10 is intended to include any pure compound or mixture of compounds predominantly aliphatic in nature and containing at least twenty carbon atoms. Petroleum wax, such as paraffin wax, is contemplated as one of the preferred sources for this heavy alkyl or wax substituent, but the invention is not limited thereto. It will be understood that when a mixture of aliphatic hydrocarbon compounds, such as those which characterize petroleum wax, is used to provide the 15 heavy alkyl substituent, the resulting composition will be an intimate admixture of compounds, or more specifically, an intimate admixture of aryl ether carboxylic acids which differ from each other with respect to the nature of the alkyl substituent. More specifically, the invention 20 contemplates an intimate admixture of alkyl substituted aroxy-aromatic carboxylic acids or an intimate admixture of alkyl substituted aroxy-aliphatic carboxylic acids wherein the acids in a given mixture differ from each other with respect to the alkyl substituents which are attached to the aryl nucleus of the aroxy group and are 25 predominantly alkyl groups of at least twenty carbon atoms, corresponding substantially to the different aliphatic hydrocarbons in paraffin wax.

In addition to the heavy alkyl or "wax" substituent and the ether acid substituent, the characterizing aryl nucleus of the compounds contemplated herein may have additional nuclear 30 hydrogen substituted with other radicals or groups. Taking this into account compounds of the type contemplated herein may be represented by the formulae



in which Z represents an aliphatic or an aromatic radical; at least one R represents an alkyl group

containing at least twenty carbon atoms and the remaining R's represent residual hydrogen or a radical selected from the group consisting of: aliphatic hydrocarbon groups having less than twenty carbon atoms, alkoxy, aroxy, aralkyl, aryl, hydroxyl, chlorine, nitro and amino radicals or groups.

In the class of these compounds or products which are preferred for use as oil addition agents it is important that the heavy alkyl (wax) substituent comprise a substantial proportion of the composition as a whole and it appears from the results of our research that there is a critical range in the degree of "wax" substitution below which the wax-substituted aryl ether acids will not satisfy the requirements for oil miscibility. This critical range in the degree of alkylation or wax-substitution may vary with: (a) the mineral oil fraction in which the product is to be used; (b) the character of the aryl nucleus (mono- or poly-cyclic); (c) mono- or poly-substitution of the aryl nucleus; and (d) other substituents which may be of positive or negative or of neutral solubilizing activity. In general it may be said that a polycyclic nucleus appears to require a higher degree of alkylation than a mono-cyclic nucleus.

In view of the foregoing variables it would be impracticable to attempt to give an expression and figure which would indicate accurately the proper degree of alkylation or heavy alkyl substitution satisfying all cases, taking these variables into account. As a guide for preparing the compound for oil improving agents our research indicates that alkylation of an aryl hydroxide with paraffin wax, to obtain the initial reactant, should be so controlled that the ratio by weight of aryl hydroxide to alkylated aryl hydroxide is not greater than about .20 or twenty percent when the weight of the aryl hydroxide component is expressed in terms of its chemically equivalent weight of phenol ( $C_6H_5OH$ ).

This ratio (which we may term the "phenolic ratio") of twenty percent, represents what we consider a maximum figure for the preferred products contemplated herein and, in general, it will be found that this figure may be lower. The actual ratio in a given case will be dependent upon the variable factors enumerated above.

The general procedure for preparing the compounds of this invention involves alkylation of an aryl hydroxide or hydroxyaromatic compound to effect substitution of the nucleus with heavy alkyl groups to the desired extent. The hydroxyl hydrogen of the alkyl substituted aryl hydroxide is then substituted with an aliphatic or aromatic carboxylic acid group.

Typical hydroxyaromatic compounds or aryl hydroxides which may be used as starting material are: phenol, resorcinol, hydroquinone, catechol, cresol, xylenol, hydroxydiphenyl, benzylphenol, phenyl-ethyl-phenol, phenol resins, methyl-hydroxy-diphenyl, guaiacol, alpha and beta naphthol, alpha and beta methyl naphthol, tolyl naphthol, xylol naphthol, benzyl naphthol, anthranol, phenyl methyl naphthol, phenanthrol, anisole, beta naphthyl methyl ether, chlorophenol, and the like. Preference in general is to the monohydroxy phenols otherwise unsubstituted, particular preference being given to phenol and alpha and beta naphthol.

The alkylation of the aryl hydroxide may be accomplished in various ways, such as by a Friedel-Crafts synthesis, using a halogenated high molecular weight aliphatic hydrocarbon

compound or mixture thereof such as chlorinated paraffin wax. Alkylation may also be effected with unsaturated high molecular weight aliphatic hydrocarbon compounds or higher alcohols in the presence of  $H_2SO_4$  as a catalyst.

Substitution of the hydroxyl hydrogen with the carboxylic acid group (Z.COOH) is conveniently accomplished by first substituting the hydroxyl hydrogen with an alkali or alkaline earth metal and then reacting the metal hydroxylate thus formed with the corresponding metal soap or salt of the desired halogenated carboxylic acid. The alkylated aryl ether carboxylic acid is finally obtained by acidifying the last obtained product with a mineral acid. Another desirable procedure for obtaining wax-aroxy-aliphatic acids is to use an ester of the aliphatic acid, instead of the metal soap or salt, and recover the acid by saponification of the final condensation product. In obtaining wax-aroxy-aromatic carboxylic acids it is preferable to use the alkali salt of a brom aromatic acid and to carry out the etherification at elevated temperature in the presence of a catalyst such as powdered copper.

Examples of the halogenated organic acids which may be used (as their alkali metal salts) in the formation of aryl ether acids are: the monobasic acids such as acetic, butyric, octoic, palmitic, stearic, naphthenic, etc.; poly-basic acids such as maleic, succinic, adipic, etc.; aromatic acids such as benzoic, phthalic, cinnamic, furoic, etc. Both the aliphatic and aromatic type acids may also carry substituents such as keto, nitro, amino, and hydroxy groups.

If it is desired to obtain a product having an aroxy or alkoxy substituent in the characterizing aryl nucleus it is preferable to start with an aryl hydroxide containing such a substituent group and effect the alkylation thereof with a high molecular weight unsaturated aliphatic hydrocarbon having a carbon chain length of at least twenty carbon atoms (such as eicosylene, ceroiene, melene, etc.) or a higher alcohol having at least twenty carbon atoms (such as ceryl alcohol, myricyl alcohol, etc.) using  $H_2SO_4$  as a catalyst.

When it is desired to obtain a nitro or amino group as an additional substituent in the characterizing aryl nucleus, the aryl hydroxide is alkylated when free of nitro or amino groups and such alkylation is followed by nitration to introduce the nitro substituent. The amino group can be obtained by reduction of the nitro group.

Further details in the procedures which may be followed in making the compositions of this invention may be obtained from the following illustrative examples.

#### 60 PREPARATION OF WAX-SUBSTITUTED PHENOXY-ALIPHATIC CARBOXYLATE SALTS

##### (1) ALKYLATION OF PHENOL

65 A paraffin wax melting at approximately 120° F. and predominantly comprised of compounds having at least twenty carbon atoms in their molecules is melted and heated to about 200° F., after which chlorine is bubbled therethrough until the wax has absorbed from sixteen per cent to twenty per cent of chlorine, such product having an average composition between a monochlor wax and a dichlor wax or corresponding roughly to a dichlor wax. Preferably the chlorination is continued until about one-fifth the weight of the

"chlorwax" formed is chlorine. A quantity of chlorwax thus obtained, containing three atomic proportions of chlorine, is heated to a temperature varying from just above its melting point to not over 150° F., and one mole of phenol ( $C_6H_5OH$ ) is admixed therewith. The mixture is heated to about 150° F., and a quantity of anhydrous aluminum chloride corresponding to about three per cent of the weight of chlorwax in the mixture is slowly added to the mixture with active stirring. The rate of addition of the aluminum chloride should be sufficiently slow to avoid violent foaming, and during such addition the temperature should be held at about 150° F. After the aluminum chloride has been added, the temperature of the mixture may be increased slowly over a period of from fifteen to twenty-five minutes to a temperature of about 250° F. and then may be more slowly increased from about 300° F. to about 350° F. If the emission of  $HCl$  gas has not ceased when the final temperature is reached, the mixture may be held at 300° or 350° F. for a short time to allow completion of the reaction. But, to avoid possible cracking of the wax, the mixture should not be heated appreciably about 350° F., nor should it be held at that temperature for any extended length of time.

It is important that all unreacted or non-alkylated hydroxyaromatic material (phenol) remaining after the alkylation reaction be removed. Such removal can be effected generally by water-washing, but it is preferable to treat the water-washed product with super-heated steam, thereby insuring complete removal of the unreacted material and accomplishing the drying of the product in the same operation.

A wax-substituted phenol prepared according to the above procedure, in which a quantity of chlorwax containing three atomic proportions of chlorine (twenty per cent chlorine in the chlorwax) is reacted with one mole of phenol, may, for brevity herein, be designated as "wax-phenol (3-20)." Parenthetical expressions of this type (A-B) will be used hereinafter in connection with the alkylated hydroxyaromatic compounds to designate (A) the number of atomic proportions of chlorine in chloraliphatic material reacted with one mole of hydroxyaromatic compound in the Friedel-Crafts reaction, and (B) the chlorine content of the chlor-aliphatic material. In the above example A=3 and B=20. This same designation will also apply to the metaloxyaromatic-metal carboxylate derivatives.

Wax-phenol (3-20) as obtained by the above procedure had a phenol content or a "phenolic ratio" of about sixteen per cent. Our research indicates that this phenolic ratio in the neighborhood of sixteen per cent may be considered as representing about the maximum for satisfactory miscibility and in viscous oils of the aryl ether acid derivatives of alkylated hydroxyaromatic compounds in which the alkyl substituent is derived from wax and the hydroxyaromatic constituent is derived from phenol ( $C_6H_5OH$ ). Effective oil-improving agents can, however, be obtained from wax-phenol (3-16), in which the phenol content or phenolic ratio is in the neighborhood of thirteen per cent.

(2) FORMATION OF WAX-SUBSTITUTED ALKALI OR ALKALINE EARTH METAL PHENATE

As an example of this step in the preparation of our oil-improving agents, 200 grams of wax phenol (12.2% combined phenol) is diluted with

600 grams of mineral oil (Say. Vis. 244 sec. at 130° F.) and reacted with 6 grams of sodium as sodium ethylate at 300° F. during a one-hour period, allowing the alcohol to distill to complete the formation of sodium phenate.

(3) FORMATION OF ETHER ACID SALTS FROM WAX-ALKALI METAL PHENATE

*Example a—Wax-phenoxyl-acetic acid*

10 24.7 grams of monochloracetic acid in 100 cc. of absolute ethyl alcohol was converted to sodium chloracetate by adding dropwise a standard alcohol solution of sodium hydroxide, maintaining the temperature of the reaction mixture below 15° F. This sodium chloracetate suspension was then added to the solution of wax sodium phenate, in mineral oil, and the reaction mixture was held at 150° F. during a two-hour period to form the wax-substituted phenoxy sodium acetate. The mixture is then neutralized with dilute hydrochloric acid to liberate the free ether acid, and is purified by water-washing the product to remove reaction salts. The product thus obtained is then dried to give a concentrated mineral oil blend of the wax-phenoxyl acetic acid. The pure undiluted acid can be obtained by use of light mineral oil such as kerosene distillate as diluent in place of the heavier distillate suggested above whereby the pure acid concentrate can be obtained by distillation of the kerosene diluent.

*Example b—Wax-phenoxyl-benzoic acid*

35 100 grams of wax phenol was reacted with 2.95 grams of metallic sodium in the presence of 5% by volume of anhydrous amyl alcohol at a temperature of 300° F. during a one hour period, allowing the alcohol to distill. The wax sodium phenate thus formed was then mixed with 28.9 grams of brom-sodium benzoate and the mixture introduced into an autoclave where it was heated, with stirring, to a temperature of about 400° F. in the presence of powdered copper as a catalyst for a period of about four hours. The product of this reaction was the sodium salt of wax phenoxy benzoic acid. The free acid was obtained by neutralizing the reaction product of the foregoing step with aqueous hydrochloric acid, followed by water washing and drying to obtain the finished product.

50 Wax-substituted aryl ether acids of the general character described above can be prepared from other wax-substituted hydroxyaromatic compounds, either mono- or poly-cyclic and substituted or unsubstituted, such, for example, as wax-naphthol (3-14) having a combined naphthol content of sixteen per cent and equivalent phenolic content or "phenolic ratio" of 10.4 per cent. They may also be obtained with other alkyl substituents than petroleum wax, although, as indicated above, alkylated hydrocarbons of the wax type (having at least twenty carbon atoms) are preferred. It is also emphasized that the invention is not limited to products obtained from acetic or benzoic acid as a source for the ether acid substituent but that any halogenated organic acid may be used in the reactions described above to obtain various ether acid substituents.

70 75 Wax-aryl ether acids of the type described above are highly viscous rubber-like products, which with the phenolic ratio properly controlled are readily soluble in mineral oils. Their color is such that they can be readily blended with light-colored mineral oil fractions without sub-

stantial darkening of the oil, which makes them particularly desirable for use in this connection.

As will appear from the foregoing description, the compounds or products may be broadly described as alkylated or wax-substituted aryl ether carboxylic acids. Ether acids derived from aliphatic acids may be characterized as alkylated or alkyl-substituted aroxy-aliphatic carboxylic acids, and those derived from aromatic acids may be characterized as alkyl or wax-substituted-aroxy-aromatic-carboxylic acids. These complex ether acids may also be defined as alkylated or wax-substituted hydroxyaromatic compounds in which the hydroxyl hydrogen has been substituted with an organic acid group, it being understood that the terms "alkyl", and "alkylated" are used herein in a broad sense to include polyatomic or polyvalent, as well as monovalent aliphatic radicals or groups; also that the term "wax" as used herein is used broadly to designate aliphatic or predominantly aliphatic materials having at least twenty carbon atoms.

We claim:

1. As a new composition of matter, an alkyl-substituted aryl ether carboxylic acid in which the alkyl substituent contains at least twenty carbon atoms, the said product possessing the property of depressing the pour point and improving the viscosity index of a mineral oil when admixed therewith in a minor proportion.

2. As a new composition of matter, an alkyl-substituted aryl ether carboxylic acid in which the alkyl substituent contains at least twenty carbon atoms and is derived from paraffin wax, the said product possessing the property of depressing the pour point and improving the viscosity index of a mineral oil when admixed therewith in a minor proportion.

3. As a new composition of matter, an alkyl-substituted aroxy aliphatic carboxylic acid in which the alkyl substituent contains at least twenty carbon atoms and is attached to the aroxy nucleus, the said product possessing the property of depressing the pour point and improving the viscosity index of a mineral oil when admixed therewith in a minor proportion.

4. As a new composition of matter, an alkyl-substituted aroxy aromatic carboxylic acid in which the alkyl substituent contains at least twenty carbon atoms and is attached to the aroxy nucleus, the said product possessing the property of depressing the pour point and improving the viscosity index of a mineral oil when admixed therewith in a minor proportion.

5. As a new composition of matter, an intimate mixture of alkyl-substituted aroxy-aliphatic carboxylic acids, said acids differing from each other with respect to the nature of the alkyl substituent, the said alkyl substituent being attached to the aryl nucleus of the aroxy group and the different alkyl substituents being predominantly alkyl groups of at least twenty carbon atoms, and having a composition corresponding substantially to the different aliphatic hydrocarbons contained in paraffin wax.

6. As a new composition of matter, an intimate mixture of alkyl-substituted aroxy-aromatic carboxylic acids, said acids differing from each other with respect to the nature of the alkyl substituent, the said alkyl substituent being attached to the aryl nucleus of the aroxy group and the different alkyl substituents being predominantly alkyl groups of at least twenty carbon atoms, and having a composition corre-

sponding substantially to the different aliphatic hydrocarbons contained in paraffin wax.

7. As a new composition of matter, an intimate mixture of alkyl-substituted phenyl ether carboxylic acids, said acids differing from each other with respect to the nature of the alkyl substituent, the said alkyl substituent being attached to the phenyl nucleus and the different alkyl substituents being predominantly alkyl groups of at least twenty carbon atoms, and having a composition corresponding substantially to the different aliphatic hydrocarbons contained in paraffin wax.

8. As a new composition of matter, an intimate mixture of alkyl-substituted phenoxy-aliphatic-carboxylic acids, said acids differing from each other with respect to the nature of the alkyl substituent, the said alkyl substituent being attached to the phenyl nucleus of the phenoxy group and the different alkyl substituents being predominantly alkyl groups of at least twenty carbon atoms, and having a composition corresponding substantially to the different aliphatic hydrocarbons contained in paraffin wax.

9. As a new composition of matter, an intimate mixture of alkyl-substituted phenoxy-acetic acids, said acids differing from each other with respect to the nature of the alkyl substituent, the said alkyl substituent being attached to the phenyl nucleus of the phenoxy group and the different alkyl substituents being predominantly alkyl groups of at least twenty carbon atoms, and having a composition corresponding substantially to the different aliphatic hydrocarbons contained in paraffin wax.

10. As a new composition of matter, an intimate mixture of alkyl-substituted phenoxy-aromatic-carboxylic acids, said acids differing from each other with respect to the nature of the alkyl substituent, the said alkyl substituent being attached to the phenyl nucleus of the phenoxy group and the different alkyl substituents being predominantly alkyl groups of at least twenty carbon atoms, and having a composition corresponding substantially to the different aliphatic hydrocarbons contained in paraffin wax.

11. As a new composition of matter, an intimate mixture of alkyl-substituted phenoxy-benzoic acids, said acids differing from each other with respect to the nature of the alkyl substituent, the said alkyl substituent being attached to the phenyl nucleus of the phenoxy group and the different alkyl substituents being predominantly alkyl groups of at least twenty carbon atoms, and having a composition corresponding substantially to the different aliphatic hydrocarbons contained in paraffin wax.

12. As a new composition of matter, an intimate mixture of alkyl-substituted aryl ether carboxylic acids, said acids differing from each other with respect to the nature of the alkyl substituent, the said substituent being attached to the aryl nucleus and the different alkyl substituents being predominantly alkyl groups of at least twenty carbon atoms, and having a composition corresponding substantially to the different aliphatic hydrocarbons contained in paraffin wax.

13. The method of synthesizing oil-miscible petroleum wax-aryl-ether acids which includes: reacting a chlorinated wax with a hydroxyaromatic compound in proportions such that the resulting wax-hydroxyaromatic compound has a hydroxyaromatic content not greater than the equivalent of about twenty per cent phenol; sub-

stituting the hydroxyl hydrogen with a metal selected from the group consisting of alkali and alkaline earth metals to form the corresponding wax-aryl-metal oxide; reacting the wax-aryl-metal oxide with the alkali metal salt of a halogenated organic acid to form the corresponding

salt of a wax-aryl-ether acid; and neutralizing said last mentioned salt with a mineral acid to form the wax-aryl-ether acid.

ORLAND M. REIFF.  
FERDINAND P. OTTO.

CERTIFICATE OF CORRECTION.

Patent No. 2,252,666.

August 12, 1941.

ORLAND M. REIFF, ET AL.

It is hereby certified that error appears in the printed specification of the above numbered patent requiring correction as follows: Page 4, second column, line 70, strike out "petroleum" and insert the same after "chlorinated" in line 71, same claim; and that the said Letters Patent should be read with this correction therein that the same may conform to the record of the case in the Patent Office.

Signed and sealed this 10th day of February, A. D. 1942.

(Seal)

Henry Van Arsdale,  
Acting Commissioner of Patents.